

April 16, 1957

F. E. GARRIOTT ET AL

2,789,065

ALUMINUM BRONZE WELD ROD

Filed Nov. 5, 1953

FIG. 1.



FIG. 2.



FIG. 3.



INVENTOR  
FRANCIS E. GARRIOTT  
JOHN F. KLEMENT  
BY

*Andrew S. Seale*  
ATTORNEYS

## 1

2,789,065

**ALUMINUM BRONZE WELD ROD**

Francis E. Garriott, West Allis, and John F. Klement, Milwaukee, Wis., assignors to Ampco Metal, Inc., Milwaukee, Wis., a corporation of Wisconsin

Application November 5, 1953, Serial No. 390,372

5 Claims. (Cl. 117—207)

This invention relates to weld rods and method of producing the same.

Extruded or rolled aluminum bronze rod having an aluminum content of less than 11% is comparatively ductile and may be readily cold drawn to size and fabricated into core wire for weld rods. However, an aluminum bronze having a higher aluminum content than 11% or having substantial additions of other alloying elements does not possess sufficient ductility to be successfully cold drawn to size. These higher alloy aluminum bronzes must be swaged to form a core wire, and this process is expensive and slow as compared with a cold drawing operation.

This invention is based on the concept that an extremely hard, high strength aluminum bronze weld deposit can be obtained by use of a weld rod or filler rod composed of a standard, cold drawable aluminum bronze core wire covered with a coating containing alloying metals which give to the resulting weld metal the particular higher hardness and tensile strength required.

By altering the composition and proportion of the alloying metals in the coating applied to the standard aluminum bronze core wire, any given hardness and tensile strength, within practical limits, can be obtained in the weld deposit.

In the past it has been proposed to introduce alloying metals into weld rod coatings to compensate for the loss of alloying elements during the arcing action due to oxidation, but the present invention proposes introducing hardening metals into the flux coating of an inexpensive, cold drawable aluminum bronze alloy rod to increase the hardness of the weld deposit.

The drawings furnished herewith illustrate the best mode presently contemplated for carrying out the invention set forth hereinafter.

In the drawings:

Figure 1 is a plan view of the weld rod of the present invention;

Fig. 2 is a transverse section taken on line 2—2 of Fig. 1; and

Fig. 3 is a perspective view of a second embodiment of the invention with parts broken away in section.

Referring to the drawings, there is shown in Figs. 1 and 2 a weld rod or electrode comprising a metal core 1 and an outer coating 2.

The core 1 is formed of an extruded or rolled aluminum bronze alloy rod which is cold drawable to size. The core, generally, may have the following compositional range:

| Percent  |         |
|----------|---------|
| Aluminum | 1—10    |
| Iron     | 0—5     |
| Nickel   | 0—5     |
| Copper   | Balance |

An aluminum bronze having an aluminum content between 1% and 10%, and the balance substantially

## 2

copper has a deposit hardness of less than 150 Brinell and may be readily drawn to size and employed as the core wire 1. However, as the aluminum content of the alloy is increased to over 10% the hardness correspondingly increases and the drawable qualities of the alloy are reduced.

A typical example of a commercially available aluminum bronze alloy which is capable of being readily drawn to size and is suitable for use as the core 1 is as follows:

| Percent  |         |
|----------|---------|
| Aluminum | 7       |
| Iron     | 2.5     |
| Copper   | Balance |

Another example of a specific alloy having a small amount of nickel and which may be drawn, is as follows:

| Percent  |         |
|----------|---------|
| Aluminum | 7       |
| Iron     | 2.5     |
| Nickel   | .25     |
| Copper   | Balance |

In order to have a core wire which is drawable and of standard composition and yet have a final weld metal composition that has higher hardness and tensile strength, metal alloying elements are employed in the coating 2. The coating consists, generally, of the usual fluxes which are compatible to the aluminum bronzes, a binder, and alloying elements which may take the form of powdered metal mixed individually with the fluxes and binder or as a pre-alloy of the alloying metals.

The coating may be applied to the core wire by dipping, extruding, spraying, or any of the usual processes by which coatings are normally applied to the core.

The alloying elements employed in the coating depend on the particular properties desired in the weld metal.

The following elements have been successfully employed in varying amounts to provide a weld metal having various degrees of hardness and strength: copper, iron, aluminum, nickel, manganese, silicon, zinc, tin, cobalt, beryllium, vanadium and chromium.

For example, if a weld deposit is desired having the following composition:

| Percent  |         |
|----------|---------|
| Aluminum | 14      |
| Iron     | 4       |
| Nickel   | .35     |
| Copper   | Balance |

a cold drawable aluminum bronze of the following composition may be employed as the core:

| Percent  |         |
|----------|---------|
| Aluminum | 10      |
| Iron     | 1       |
| Nickel   | .10     |
| Copper   | Balance |

Sufficient additions of aluminum, iron and nickel are mixed with the weld rod coating to increase the concentrations of these metals to the desired level in the weld deposit. The exact amount of aluminum, iron and nickel added to the coating depends on numerous factors such as, the diameter of the core, the thickness of the coating, etc. and is usually determined by a trial and error process after a preliminary determination of the approximate weight relationships. Generally, the metal alloying elements may comprise up to 50% by weight of the wet coating and an excess of about 10%, by weight, of the theoretically required amount of metal additions is added to the coating to compensate for melt loss.

The following core compositions have been employed to obtain the following respective weld deposits:

|   |         | Al   | Fe  | Si  | Ni   | Cu      |
|---|---------|------|-----|-----|------|---------|
| 1 | Core    | 7.5  |     |     |      | Balance |
|   | Deposit | 9.0  | 2.9 | 1.5 |      | Do.     |
| 2 | Core    | 9.5  | 0.8 | 0.1 |      | Do.     |
|   | Deposit | 11.0 | 3.8 | 1.5 |      | Do.     |
| 3 | Core    | 7.0  | 2.5 |     | 2.25 | Do.     |
|   | Deposit | 10.5 | 4.0 |     | 1.00 | Do.     |

Numerous modifications of the above compositions have been made producing satisfactory results.

The flux coating generally, consists of fluxing agents such as sodium fluoride or cryolite to remove the oxides formed in the melting process; gas-shielding and reducing materials, such as carbon and alpha flock, to provide protection against excessive oxidation, and a binder, such as sodium or potassium silicate, to bind the ingredients together and control the surface tension of the slag.

The metal alloying elements may be employed in the coating as individual metals or as a pre-alloy.

To prepare a pre-alloy, the desired metals are melted together and cooled. The resulting pre-alloy is then ground to a powdered form and mixed with the flux. The pre-alloy should be sufficiently refractory so that it will break up easily into a proper particle size and be readily distributed throughout the coating. Copper is sometimes employed in the pre-alloy to give the pre-alloy the required refractory properties.

To fabricate the weld rod, the standard aluminum bronze core wire is initially drawn to size. The coating is prepared by mixing the individual metals or the pre-alloy with the flux and binder. Water is added to the mixture to provide the coating with the proper consistency to enable it to be applied to the core wire.

The coating is then applied to the core wire by dipping, extruding, or any other conventional process, and the coating is then permitted to set at room temperature for a short period of time. After setting, the weld rod is heated at a temperature of about 550° F. for a period of about two hours.

Fig. 3 illustrates a modified form of the invention. The weld rod comprises a cold drawable aluminum bronze core 3, similar in composition and properties to core 1 of the first embodiment, and an aluminum alloy sheath 4.

The cold drawable core has the following general composition by weight:

|          | Percent |
|----------|---------|
| Aluminum | 1-10    |
| Iron     | 0-5     |
| Nickel   | 0-5     |
| Copper   | Balance |

The deposit hardness of the core 3 having the above composition is generally less than 150 Brinell and the aluminum alloy sheath serves to produce a final weld deposit hardness in excess of that of the cold drawable core.

The sheath 4 has the following general composition by weight:

|           | Percent |
|-----------|---------|
| Aluminum  | 90-100  |
| Copper    | 0-5     |
| Silicon   | 0-5     |
| Manganese | 0-2.5   |
| Chromium  | 0-3     |
| Nickel    | 0-2     |

The weight relationship between the sheath 4 and the core 3 depends on the particular hardness and tensile strength desired in the weld deposit. As in the case of the first embodiment, the approximate weight relationships of core and sheath are determined for a desired weld deposit composition and the precise relationships are then determined on a trial-and-error basis.

The sheath may be applied to the core in any conventional manner. A very satisfactory method of application is a combined wrapping and drawing operation where the sheath is wrapped around the oversize core and the composite structure is drawn to size. The sheath metals may also be applied to the core by electroplating.

If the weld rod is to be employed as a consumable electrode in a welding gun or the like, no flux coating is required. However, a flux coating, without the addition of powdered metals, may be applied to the sheath if the weld rod is to be used in other applications where a flux coating is desirable.

Generally a cold drawable aluminum bronze having up to 10% aluminum to be employed as the core has a deposit hardness of less than 150 Brinell (3000 kg. load). With the use of the present invention the hardness of the weld deposit can be increased to over 160 Brinell and to about 300 Brinell with the metal-arc and carbon-arc welding processes and to about 340 Brinell with inert gas processes due to the increased shielding effect of argon and helium gases.

The present invention provides a very convenient method of producing a weld metal having a high hardness and tensile strength by using a standard drawable core wire. A core wire of a standard composition may be employed and the composition of the weld metal may be varied for any particular welding operation by merely varying the amount and nature of the alloying elements in the coating.

Various modes of carrying out the invention are contemplated as within the scope of the following claims which particularly point out and distinctly claim the subject matter regarded as the invention.

We claim:

1. A weld rod comprising a core consisting of about 1 to 10% aluminum, up to 5% iron, up to 5% nickel and the balance being substantially all copper and having a deposit hardness of less than 150 Brinell, and a metal sheath applied to the outer surface of said core and comprising over 90% aluminum, up to 5% copper, up to 5% silicon, up to 2.5% manganese, up to 3% chromium and up to 2% nickel, said sheath alloying with the core during welding to produce a weld deposit having a hardness in excess of 160 Brinell.

2. An electrode comprising a core consisting of about 1 to 10% aluminum and the balance being substantially all copper and having a deposit hardness of less than 150 Brinell, and a coating applied to the outer surface of said core and having metal alloy additions therein, said alloy additions consisting of at least 90% aluminum, up to 5% copper, up to 5% silicon, up to 2.5% manganese, up to 3% chromium and up to 2% nickel, said alloy additions alloying with the core during welding to produce a weld deposit having a hardness in excess of 160 Brinell.

3. A weld rod comprising an aluminum bronze core consisting of about 1 to 10% aluminum and the balance substantially all copper and having a deposit hardness of less than 150 Brinell under predetermined welding conditions, and coating containing hardening additions selected from the group consisting of aluminum, iron and silicon and applied to the outer surface of the core, said additions being present in excess of the amount of said hardening additions lost during the melt and in sufficient amount to provide the weld rod with a deposit hardness of over 160 Brinell under the same welding conditions.

4. A weld rod comprising a core consisting of about 1 to 10% aluminum, up to 5% iron, up to 5% nickel and the balance being substantially all copper and having a deposit hardness of less than 150 Brinell under predetermined welding conditions, and a flux coating applied to the outer surface of said core and containing metal hardening additions selected from the group consisting of aluminum, iron and silicon, said additions being present

in excess of the amount of said metal additions lost dur-

ing the melt and in sufficient amount to provide the weld rod with a deposit hardness of about 300 Brinell under the same welding conditions.

5. A weld rod comprising a core consisting of about 1 to 10% aluminum, up to 5% iron, up to 5% nickel and the balance being substantially all copper and having a deposit hardness of less than 150 Brinell under predetermined welding conditions, and a coating applied to the core and comprising fluxing material, carbonaceous material, alloy material and a binder, said alloy material comprising minor amounts of metals selected from the group consisting of iron, nickel, silicon, manganese, vanadium and chromium and the balance of said alloy material being aluminum, said alloy material being present

in sufficient amount to provide the weld rod with a deposit hardness of over 160 Brinell under the same welding conditions.

References Cited in the file of this patent

UNITED STATES PATENTS

|           |               |       |               |
|-----------|---------------|-------|---------------|
| 2,238,392 | Matush        | ----- | Apr. 15, 1941 |
| 2,408,619 | Friedlander   | ----- | Oct. 1, 1946  |
| 2,430,419 | Edens         | ----- | Nov. 4, 1947  |
| 2,464,836 | Thomas et al. | ----- | Mar. 22, 1949 |

FOREIGN PATENTS

|         |               |       |              |
|---------|---------------|-------|--------------|
| 613,737 | Great Britain | ----- | Dec. 2, 1948 |
|---------|---------------|-------|--------------|